

## UNITED STATES PATENT OFFICE

2,015,201

PRECIPITATING BATH FOR VISCOSE  
FILAMENTS

Johann Joseph Stöckly and August Brötz, Tel-tow-Seehof, Germany, assignors to North American Rayon Corporation, New York, N. Y., a corporation of Delaware

No Drawing. Application July 15, 1930, Serial No. 468,197. In Germany July 15, 1929

## 3 Claims. (Cl. 18—54)

In the use of sulphuric acid—sodium sulphate baths as precipitating means for extruded filaments, it is well known that particularly desirable products are obtained if the sodium sulphate is present in a sufficient quantity to overcome the bi-sulphate reaction from the sulphuric acid present. In order to prevent loss of lustre and softness and shrinking of the filaments, the use of the processes now known necessitate the application of tension to the filaments during the washing and first drying step. This is indicated by the usual method of washing and drying the filaments while they are on the fixed take-up devices, in the spool spinning, and glass-roller spinning machines. When the so called centrifugal spinning process is used, installations of stretching trucks, or the addition of other elements, is necessary.

According to the present invention, the use for any of these spools, glass-rollers, stretching or stiffening devices, etc., is done away with, and are not necessary in and treating (especially drying) the newly spun filaments. When the well known Mueller bath discussed in paragraph one, is used, together with the abridged treatment later described the two bath ingredients above do not prevent shrinkage, loss of lustre and softness, etc. The use of a higher concentration of the salt solution will improve matters to a slight degree, but crystallization of the salts with consequent damage to the filaments, may result.

The present invention contemplates the addition of certain quantities of zinc sulphate to the bath, this addition producing good results in obviating the defects above mentioned. Experience, however, has shown that despite the addition of zinc sulphate, the sulphate concentration of the bath must not sink below a certain minimum percentage of sulphuric acid present, if good results are to be obtained. Further, it has been discovered that the sodium sulphate concentration must not be allowed to drop to less than about 230 gr.  $\text{Na}_2\text{SO}_4$  per liter. Although the concentration of sodium sulphate may be increased, the best results are obtained when about 250 gr.  $\text{Na}_2\text{SO}_4$  per liter are used.

The addition of the zinc sulphate, and the quantity of this salt to be added, is important. For the best results, at least 5 gr./litre of  $\text{ZnSO}_4$  should be present, although the exact percentage present is dependent upon the concentration of sulphuric acid used.

As a general rule, higher concentrations of sulphuric acid necessitate the use of larger percentages of zinc sulphate. For example, it has been

found that when 100 grs.  $\text{H}_2\text{SO}_4$  per liter and 250 gr.  $\text{Na}_2\text{SO}_4$  per liter are used, 10 gr. of  $\text{ZnSO}_4$  must be added to give the best results. Similarly, for 110 gr.  $\text{H}_2\text{SO}_4$  per liter, 15 gr.  $\text{ZnSO}_4$  per liter are necessary. When still higher concentration of sulphuric acid is used, for instance, 135 gr.  $\text{H}_2\text{SO}_4$  per liter, 25 gr.  $\text{ZnSO}_4$  per liter are necessary.

The addition of too great a percentage of  $\text{ZnSO}_4$  makes it necessary that the filaments contact with the bath for a longer period of time. Otherwise, incomplete coagulation of the filaments results in their agglutination. This latter difficulty may be overcome or prevented by acidifying the newly spun thread before washing and drying.

This new process may be advantageously used with the centrifugal spinning method. The newly spun cakes are reeled in a wet and acidic condition, and then washed in suitable washing machines, treated, and hung up freely to dry. In this manner it is possible by eliminating the first washing and first drying, to obtain the skeins in one stroke. In spite of this shortened process the yarn is not unduly shrunk, and possesses the desired lustre and softness.

Another advantage may arise from using this new process in the centrifugal spinning method. The newly spun cakes may be washed, desulphurized, bleached, soaped, scoured, etc., without the use of any stiffening bodies, and these cakes may then be dried and used for various purposes without the necessity of using any stiffening bodies, or stretching.

35

## Example

Normal viscose containing 7% cellulose and 7% alkali, aged from 9—10° Hottenroth, is spun into artificial silk of 120 denier, 5 denier to the single filament, by use of the usual metallic or non-metallic spinnerettes. The following spinning bath is used;

110 gr.  $\text{H}_2\text{SO}_4$  per liter,  
250 gr.  $\text{Na}_2\text{SO}_4$  per liter,  
15 gr.  $\text{ZnSO}_4$  per liter,  
dipping distance 20 cm.

45

If the machine used is the well known centrifugal spinning machine, the spun cakes are at once reeled in their wet and acidic condition, then thoroughly washed and dried without stretching. This method produces a lustrous, soft, and not unduly shrunk yarn, especially when the desulphurization step is completed.

We claim:

55

1. In a process for the manufacture of artificial filaments, yarns, threads, etc., from a viscose solution, the steps of preparing a normal viscose solution, and spinning it into a bath containing:

|                 |          |
|-----------------|----------|
| 5               | Gr/litre |
| Sulphuric acid  | 110      |
| Sodium sulphate | 250      |
| Zinc sulphate   | 15       |

10 and then washing, after-treating and drying the filaments, yarn, etc., in an unstretched condition.

2. In a process for the manufacture of artificial filaments, yarns, threads, etc., from a viscose solution, the steps of preparing a normal viscose solution, and spinning it into a bath containing:

|                 |                |
|-----------------|----------------|
| 15              | Per cent       |
| Sulphuric acid  | 8.25 to 10.71  |
| Sodium sulphate | 18.75 to 19.82 |
| Zinc sulphate   | 0.825 to 1.98  |

and then washing, after-treating and drying the filaments, yarn, etc., in an unstretched condition.

3. In a process for the manufacture of artificial filaments, yarns, threads, and the like, the steps of preparing a normal viscose solution and extruding the said solution into a bath containing the following constituents in the quantities indicated:

|                 |             |
|-----------------|-------------|
| 5               | Grams/liter |
| Sulphuric acid  | 100         |
| Sodium sulphate | 230         |
| Zinc sulphate   | 10          |

and then treating the freshly extruded product and drying it without the application of such tension as would cause stretching.

JOHANN JOSEPH STÖCKLY.  
AUGUST BRÖTZ.